

## UNITED STATES PATENT OFFICE.

HENRY PHILIP SHOPNECK, OF DORCHESTER, MASSACHUSETTS.

## IMPREGNATED SHOE STIFFENER.

No Drawing.

Application filed February 14, 1927. Serial No. 169,241.

- This invention relates to the manufacture of impregnated felt, and more especially, to the manufacture of felts stiffened by impregnation with celluloid.
- 5 Felts impregnated with celluloid have been found to be very useful in the shoe industry. Such stiffened materials have been used for box toes, counters, and, more recently, inner-soles in the manufacture of shoes.
- 10 The felt base usually employed in preparing such stiffeners is a villous pile fabric, which, although yielding a very good and desirable product, is very expensive, and it has been the aim of box toe and counter manufacturers to secure a substitute material capable of being used in substantially the same manner in the process of manufacturing box toes and counters for use in shoes, but less expensive in cost of manufacture.
- 15 20 Various substitutes have been proposed, among them being such products as short-fibred roofing felt, puffed paper, and cotton-lined pulp products. All such materials have failed primarily because they were not sufficiently absorbent to insure the retention of a prepondering amount of celluloid, and also because of the papery nature of the impregnated product.
- 25 After many experiments, I have finally succeeded in preparing an impregnated felt which meets with all of the requirements of shoe-stiffener and shoe manufacture.
- 30 In carrying out my invention I take a relatively short fibrous pulp, such as textile rags (mixed cotton and wool rags), or a mixture of such rags and other fibres such as cellulosic pulps, asbestos, with or without inert filling substances such as clay, celite, and so forth, and treat it, in the presence of water, in a beater engine, or hollander, until all of the fibres have been brushed out smoothly. I then add relatively longer fibres, such as jute, hair, silk, and/or other long fibres, and crush out the mixture without, however, cutting the long fibres. After mixing the stock with a large volume of water, I sheet it out and dry it on a cylinder machine.
- 35 40 45 By the term "long fibre" I mean to identify a fibre much longer than the usual length run on cylinder machines. The usual length of fibre incorporated in felts run on cylinder machines is about four millimeters, and by the term "long fibre" is meant fibres varying in length from six or seven millimeters to twenty millimeters or more.
- The textile rags are usually finely shredded before being loaded into the beater engine, this being found to yield a smoother felt than the usual practice of coarsely cutting the textile rags. The long fibres are obtained from various sources, and undergo various treatments, depending on the particular class of fibre, before adding to the beaten shorter fibres. When long hair is used, it is first washed free of lime, and is then added directly to the beater engine. On the other hand, when silk, jute, or wool fibre is added to supply the longer fibre, the silk cloth, jute bagging, or wool flock, containing the respective fibres, are first loosely fiberized, preferably by means of a textile picking machine, yielding a fibre about an inch long.
- The method of impregnating the felt with celluloid generally consists in dissolving scrap celluloid trimmings or waste film in various solvents, of which a mixture of equal parts of di-acetone and grain alcohol is an example, and then dipping the felt in the viscous solution so formed, scraping off or squeezing out the excess solution, and then spraying with or dipping the felt in water.
- The product resulting from the impregnation of such long fibred felts with celluloid is quite dense, and may be used for various purposes. When used for box toes for shoes, it is first softened by means of solvents, of which a mixture of equal parts of grain alcohol and di-acetone is an example, and is then lasted with the toe portion of the upper, together with the lining, so as to conform to the shape of the last, and hardens and sets when the solvent evaporates. Likewise, it may be used for counters for shoes, and also for inner-soles. Being inexpensive to manufacture, it permits of wide use in many different industries. The combination of the celluloid and felt containing a portion of long-fibred threads distributed throughout a sort-fibred base represents a new composition of matter having very many uses and yet is inexpensive to manufacture.
- 50 55 60 65 70 75 80 85 90 95 100 105 110 As an example of the proportions of materials and substances used in preparing the impregnated felt, I cite the following: 1150 pounds of shredded or picked textile rags, containing equal parts of cotton and wool, are loaded into a beating engine together with sufficient water to promote circulation. The stock is beaten out until smooth, and then 350 pounds of picked jute or silk

threads, or washed hair, is added, and mixed in the engine until it is evenly distributed. The stock is then mixed with more water, pumped to a Jordan engine, and finally 5 sheeted out and dried on a cylinder machine. The impregnating bath may be prepared by dissolving 600 pounds of celluloid trimmings in 3400 pounds of solvent containing equal weights of grain alcohol and diacetone. 10 Various modifications in materials, proportions, and methods of impregnating may obviously be resorted to, but all such variants are to be considered to be within the scope of my invention as defined in the appended 15 claims.

What I therefore claim and desire to secure by Letters Patent is:

1. A felted material of the water-laid type for making box toes of shoes, comprising, in 20 combination, a sheet formed, substantially, of a short fibrous pulp, having relatively longer fibres distributed therethrough, and

in felted relation therewith, and a celluloid impregnating agent, said sheet impregnated with said celluloid. 25

2. A felted material of the water-laid type, for making box toes of shoes, comprising in combination, a sheet formed, substantially, of a short, fibrous pulp, having relatively longer silk fibres distributed therethrough, and in felted relation therewith, and a celluloid impregnating agent, said sheet being saturated with said celluloid. 30

3. A felted material, of the water-laid type, for making box toes of shoes, comprising, in combination, a sheet formed, substantially, of short-beaten textile rags, having relatively longer fibres distributed therethrough, and in felted relation therewith, and a celluloid impregnating agent, said sheet 35 being impregnated with said celluloid. 40

In testimony whereof I affix my signature.

HENRY PHILIP SHOPNECK.